

1

3,108,897

**PROCESS FOR COLORING GLASS FABRICS**  
William L. Hamiter and Jimmy M. Collins, Statesville,  
N.C., assignors to United Merchants and Manufacturers,  
Inc., New York, N.Y., a corporation of Delaware  
No Drawing. Filed May 26, 1960, Ser. No. 31,838  
11 Claims. (Cl. 117—37)

This invention relates to the coloring or dyeing of fabrics having different surface structure or characteristics to obtain different tone effects.

Among the fabrics which may be dyed by the present invention are glass fiber fabrics, particularly those woven from glass yarns of lime-alumina-borosilicate relatively alkali free; fabrics made from cellulosic fibers, including cotton, rayon, cellulose acetate, and other cellulosic fibers; wool; silk; synthetic fabrics such as those prepared from acrylic (e.g. Orlon, Creslan, Acrilan, Varel, Zefran, Darvan and Dynel), polyester (e.g., ethylene glycol-terephthalic acid condensation polymers such as Dacron), polyamide (nylon), vinyl and vinylidene (e.g., Saran) fibers, polyethylene and polypropylene; and blends of two or more of any of the fibers enumerated above.

Fabrics of different surface structure or characteristics may be produced by any known procedure. For example, the fabrics may be woven from textured, nubbed, loop, knot, slub, bulked, bouclé, taslan, or filament-type yarns to produce loosely woven areas and tightly woven areas. The fabrics may be woven to produce a base having throws or loops thereon and thus provide two different surface structures or characteristics, one the base, and the other the throws or loops thereon. Fabrics may be woven in a conventional manner to provide a uniformly woven fabric and then napped to produce different surface characteristics. For example, a cotton fabric (100% cotton) or one woven from a blend of cotton and other fibers, after de-sizing, washing, bleaching and drying, as customary, is padded through a conventional softening bath, dried, printed in selected areas with a resin-resist formulation (e.g., 34% vinyl-acrylic copolymer, 5% melamine-formaldehyde resin, 32% sodium alginate containing 4% solids, 2% amine-hydrochloride catalyst, and the rest water), which formulation, if desired, contains dyes or pigments. Other areas are then printed with printing pastes containing dyes or pigments, but no resist, and still other areas, if desired, are left unprinted. The thus treated fabric is then passed through a flat calendar at 120° F. and loop cured for three minutes at about 320° F. It is thereafter napped by passage through a napping machine of any conventional type. The areas which were resist-printed remain flat and unaltered; the remaining areas are napped to produce a three-dimensional raised pattern thus forming a fabric having different surface structures or characteristics, one of which is the napped areas and the other the resist-printed areas.

Still another example of fabrics having different surface characteristics are flocked fabrics in which the flocking is applied to produce design or pattern effects. In such fabrics, the unflocked base fabric has one surface characteristic and the flocked areas another surface characteristic provided by the flocking.

This invention is particularly concerned with the dyeing of glass fiber fabrics. Heretofore, to produce glass fiber fabrics having dyed pattern effects, bulked yarns have been pre-dyed in two or more colors and woven in the desired pattern. This requires several time-consuming operations including the steps of pre-dyeing the yarn, weav-

2

ing and finishing the pre-dyed yarn. These operations require the production of different batches of selected dyed yarns for each fabric pattern or style, which unnecessarily complicates the weave mill operations with consequent increased cost of producing the finished fabrics.

It is among the objects of the present invention to provide a process for selectively coloring or dyeing fabrics having different surface structures or characteristics to produce different tonal effects without the complications and consequent additional expenses, inherent in pre-dyeing the yarn, weaving and finishing the pre-dyed yarn.

A further object of the invention is to provide such a process for dyeing fabrics woven from textured, bulked, bouclé, taslan or filament type yarns, including glass fiber yarns, which process produces fabric pattern effects by selectively dyeing certain areas of the fabric, namely, the loosely constructed or float areas in preference to the more tightly constructed areas, usually the background areas thereof.

Still another object of this invention is to provide a process for dyeing fabrics having different surface characteristics involving the utilization of one and the same dye bath to produce different color effects on these fabrics, for example, to dye the base, background, or tightly woven areas one color while dyeing the float, throw, loop, or other areas of different surface characteristics a different color.

Other objects and advantages of the present invention will be obvious from the following detailed description thereof.

The process of this invention involves mixing a cationic flocculating agent with a dispersion of a pigment to produce a dispersion containing flocculated pigment particles and treating a fabric having different surface characteristics with this dispersion. This treatment results in the flocculated pigment particles dyeing the loosely constructed, float, raised or bulked areas of the fabric in preference to or to the exclusion of the areas of the fabric having different surface characteristics, e.g., the tightly constructed or background areas.

The dyeing bath used in the practice of the process of this invention comprises a dispersion of a pigment, including all or a substantial proportion of the pigment particles in agglomerated or flocculated form due to the addition of the cationic flocculating agent.

While anionic pigment dispersions are preferred, any pigment which can be charged anionically, can be used. Thus dry powdered pigments which can be charged anionically may be employed. In the presence of an anionic binder in the dye bath employed with such pigments, the pigments acquire an anionic charge and agglomerate upon addition of the cationic flocculating agent. In general, the pigment particles should have a particle size (the largest dimension of the individual particles) within the range of from 0.007 to 40 microns. In the case of oxide pigments the particle size is usually within the range of from 0.2 to 15 microns. The concentration of the pigments in the dye bath should be from 0.02 to 5%, preferably 0.05 to 4% by weight based upon the total weight of the bath.

Pigments useful in the practice of this invention are the inorganic pigments, chiefly the oxides, sulfites and sulfates of cobalt, chromium, aluminum, iron, zinc, cadmium, manganese, and selenium and organic pigments such as the phthalocyanine dyes; anthraquinone, thioindigo, and indanthren vat dyes; azo coupling dyes; Hansa yellow and carbon black.

Examples of such pigments are given in Table I which follows:

TABLE I

| Trade name:                                                                                             | Classification                                                                                           |
|---------------------------------------------------------------------------------------------------------|----------------------------------------------------------------------------------------------------------|
| Interchemical Corporation's—<br>Padding Brown 9500-21<br>Padding Brown<br>R 9550-1                      | Indanthren Vat type.                                                                                     |
| Padding Yellow N 9851<br>Padding Yellow K 9850<br>Padding Green B 9450<br>Padding Violet<br>4B 9652     | Iron Oxide Red,<br>Indanthren Vat type.<br>Iron Oxide Yellow.<br>Phthalocyanine.<br>Indanthren Vat type. |
| Padding Red FG 9352<br>Padding Orange<br>2R 9800-16                                                     | Indanthren Vat type.<br>Molybdate Orange type.                                                           |
| Padding Chartreuse<br>9852                                                                              | Lithosol Fast Yellow 3DB.                                                                                |
| Padding Grey 2R 9250<br>Padding Blue 2G 9750                                                            | Carbon Black.<br>Phthalocyanine.                                                                         |
| Kentucky Color & Chemical Company's—<br>Cadmium Selenide Red<br>WDP 10-73K<br>Red Oxide                 | Cadmium Red.                                                                                             |
| WDP 10-9951<br>Cadmium Yellow Lemon<br>WDP 20-1575<br>Yellow Iron Oxide<br>WDP 20-8871                  | Iron Oxide Red.<br>Cadmium Yellow.<br>Iron Oxide Yellow.                                                 |
| Chromium Oxide<br>WDP 30-9906<br>Phthalocyanine Green<br>WDP 30-3820<br>Burnt Umber                     | Chromium Oxide Green.<br>Phthalocyanine.<br>Iron Oxide Brown.                                            |
| WDP 50-0525<br>Phthalocyanine Blue<br>WDP 41-4852                                                       | Phthalocyanine.                                                                                          |
| du Pont's—<br>Ponsol Yellow AR dbl<br>paste                                                             | Anthraquinone Vat type.                                                                                  |
| Arnold Hoffman Company's—<br>Ahecovat Olive T paste<br>Ahecovat Jade Green B<br>Ahecovat Olive Green BL | Anthraquinone Vat type.<br>Anthraquinone Vat type.<br>Anthraquinone Vat type.                            |
| Ciba's—<br>Cibanone Brown 3B<br>Cibanone Black DRB<br>Microfix Golden Yellow<br>G                       | Anthraquinone Vat type.<br>Anthraquinone Vat type.<br>Anthraquinone Vat type.                            |
| American Aniline's—<br>Amanthrene Dark Brown<br>BW                                                      | Indanthrene Vat type.                                                                                    |
| Putnam's—<br>Lumatex Brilliant<br>Orange G                                                              | Anthraquinone Vat.                                                                                       |
| Lumatex Dark Brown T<br>Lumatex Brilliant<br>Yellow                                                     | Iron Oxide.                                                                                              |
| Lumatex Scarlet B<br>Lumatex Yellow Brown<br>G                                                          | Azo-coupling.<br>Azo-coupling.<br>Iron Oxide.                                                            |
| Sandoz—<br>Graphitol Blue 6806-2<br>Graphitol Yellow 4882-2<br>Graphitol Black<br>Graphitol Brown G     | Phthalocyanine.<br>Hansa Yellow.<br>Carbon Black.<br>Thioindigoid Vat.                                   |

The oxides, sulfites and sulfates of cobalt, chromium, aluminum, iron, zinc, cadmium, manganese and selenium sold by B. F. Drakenfeld Company, for example, the products sold by them under their trade names:

Egyptian Blue 10012  
Yellow Brown 10017  
Deep Yellow 10058  
Turquoise 10119  
Deep Brown 10184  
Burgundy 10176

The preferred cationic flocculating agent employed in the dyeing bath is deacetylated chitin (polymeric acetamino carbohydrate), which is preferably employed in dilute acidic aqueous solution. This material may be obtained by heating crude chitin successively with soda ash and hydrochloric acid to remove the lime salts and adherent protein followed by digesting the sodium hydroxide or other alkali at an elevated temperature under conditions excluding oxidation, to produce deacetylated chitin. The deacetylated chitin thus produced is reacted with aqueous acetic acid, producing the water-soluble acetic acid salt. While it is preferred to use the acetic acid salt, other salts may be used such as, for example, those formed by reacting the purified deacetylated chitin with formic, pyruvic, or lactic acid. For a more detailed description of the production of such acid salts of deacetylated chitin, reference may be had to United States Patents 2,040,879 and 2,040,880, granted May 19, 1936.

Other cationic flocculating agents may be used, however, including for example, polyalkyl-polyamines (Sandofix WE sold by Sandoz, Inc.); polyalkyl-polyamine fatty acid reaction products (Ceranine HC(A) sold by Sandoz, Inc.); amino aldehyde condensate dye-fixatives (Lyofix EW, sold by Ciba); methylchloride quaternary of the stearic acid amide of 1-(2-aminoethyl) 2-heptadecenyl-2-imidazoline (Nalco D-1535 sold by Nalco Chemical Company); fluid oil in water type emulsions of low molecular weight polyethylene chemically stabilized with a cationic amine acetate derivative of a long chain fatty compound (Moropol A-164); dicyandiamide formaldehyde dye fixatives (Umefix F sold by Valchem); products of straight chain poly-functional amines and an aldehyde such, for example, as urea formaldehyde resins modified with (a) polyamines including ethylenediamine, diethylenetriamine, tetraethylenepentamine, guanidine, phenylbiguanide, or bisguanidine, (b) hydroxylamines such as monoethanolamine or diethanolamine; (c) cyanoamines such as dicyandiamide, polyphenylbiguanide or polyphenyl methyl biguanide, (d) amino-amides such as guanidine, or (e) quaternary ammonium salts such as tetraethanol ammonium chloride, and methylated dimethyl aniline quaternary ammonium salts; and the reaction products of these resin-modifying agents with formaldehyde, in the absence of urea, such as tetraethylenepentamine-formaldehyde, bisbiguanidine-formaldehyde, polyphenolbiguanide-formaldehyde and guanylurea-formaldehyde.

The cationic flocculating agent is included in the bath in concentrations of from 0.005 to 5% based on the weight of the bath, preferably from 0.05 to 1%. The Lyofix EW may be used alone in amounts of 0.1% to 2% of the bath or with the addition of small amounts of the deacetylated chitin, particularly when dyeing the loose float areas of an all-filament yarn glass fabric. The use of Lyofix EW results in relatively small agglomerates of the pigment, particularly desirable in dyeing all-filament yarn fabrics. Upon the agglomeration of the dispersed pigment, or pigment and finish constituents present, agglomerates or flocculated particles having an average particle size of from about 10 microns to 2,000 microns result. The particle size of the agglomerates seldom exceeds about  $\frac{1}{8}$  of an inch.

The concentration of the cationic flocculating agent within the range hereinabove given depends chiefly upon the specific pigments employed in the dyeing bath, the rate of addition of the flocculating agent to the bath, the amount thereof added, the other constituents, if any, and the concentration thereof present in the dyeing bath, the bath temperature, the pH of the bath, the type of fabric dyed, and the degree of flocculation desired. While it is preferred to operate at atmospheric temperature conditions (65-105° F.), the temperature of the bath may be within the range of 35-200° F., or even higher, but below the boiling point of the lowest boiling constituent of the bath, usually the liquid.

The pH of the bath, produced by mixing the pigment, water, or other liquid and other additives and before the addition of the agglomerating agent, is within the range of 9 to 10.5. Should the pH fall below 9.5, ammonia is added to bring the pH within this range. Upon addition of Kylan or other acid agglomerating agent to a portion of this bath, say 20 to 40% by volume, the pH of this portion is usually within the range of 4.5 to 7.5. The pH of this portion, thus produced, is not critical. Upon remixing this portion with the remainder of the volume, a bath results having a pH of from 5 to 10.5. It is preferred to operate with an alkaline bath because the agglomerate dispersions are more stable under these pH conditions. On the acid side, the dispersion of agglomerates are relatively unstable; the greater the acidity the more unstable the agglomerate dispersion. Baths having a pH above 5.5 have been found satisfactory but, as noted, it is pre-

ferred to have the pH of the bath above 7. Ammonia is added for this purpose, if found necessary, to adjust the pH of the bath.

The optimum amount of cationic flocculating agent incorporated in the bath, desirably, is determined by adding predetermined amounts of the agent to be used to the dispersion of the pigment, applying the resultant dispersion by padding on a small sample of the fabric to be colored, and determining which concentration gives the desired shade.

The bath contains, in addition to the pigment and flocculating agent, a resinous film-forming binder for bonding the pigments to the fibers of the fabric to form fast colors. Any non-ionic or anionic film-forming material capable of dispersing in the liquid medium of the bath and providing an adherent pigment coating is employed. Examples of such binder resins include butadiene-acrylonitrile copolymers, such as Chemigum 248; polyethyl acrylate, Hycar 4501 (a product of the B. F. Goodrich Chemical Company); butadiene-styrene resins, (Dow Latex 762-W); dimethylol ethylene urea resins, Umac EU (a product of Valchem); dimethylol triazone resins, Stanset 125 (a product of Standard Chemical Products Co.); polyvinyl chloride; polyvinyl acetate; polyvinyl alcohol; melamine-formaldehyde resins; acrylic resins, such as methyl methacrylate, ethyl methacrylate, butyl methacrylate, ethyl acrylate, ethyl methacrylate and copolymers of these acrylates and methacrylates including, for example, the acrylic acid ester polymers, copolymers sold by Rohm & Haas Company under their trade names Rhoplex FRN, WN-75, and Rhoplex AC-33; and water-insoluble linear copolymers, or salts thereof, of monoethylenically unsaturated monomeric units comprising 0.5 to 10 percent by weight of units containing carboxyl groups; the preferred salts are the ammonium salts, or salts of the water-soluble amines, such as methylamine, diethylamine, triethylamine, mono-, di-, or triethanolamine, morpholine, etc. (Rhoplex B-15). When dry pigment capable of being charged anionically is employed, the binder resin should be an anionic resin which will in effect impart an anionic charge to the pigment and result in the formation of agglomerates containing the pigment or pigments and binder resin. The amount of binder resin incorporated in the bath is from 0.25 to 5%, preferably from 0.5 to 2% by weight based on the weight of the bath.

In addition to the pigment, cationic flocculating agent and binder resin, the bath may contain conventional materials depending upon the fabric dyed, such as softeners, delustering agents, abrasive resistant agents, and agents to impart the desired finish. For example, when dyeing glass fiber fabrics, the bath may contain a dispersion of colloidal silica in amounts ranging from 0.3 to 4%, preferably from 0.6 to 2% solids present, based on the weight of the bath, to impart a non-slip and delustering finish to the fabric. It may also contain from 0.5 to 5% solids based upon the weight of the bath of an abrasion-resistant additive, such as polytetrafluoroethylene (Teflon).

While passing the fabric through the bath, the latter is maintained in a state of agitation by any suitable means, for example, a suitable mechanical agitator, or by bubbling an inert gas through the bath. Such agitation maintains the pigment particles, including the agglomerates, dispersed throughout the bath.

While aqueous dye baths are preferred, the invention includes dye baths of other liquid media in which the pigment may be dispersed and which media, for all practical purposes, are chemically inert to the fabric being dyed and to the other constituents of the dye bath, including the cationic flocculating agent and the resin binder. Methanol, ethanol, isopropyl alcohol, and acetone are suitable media.

The constituents of the bath are mixed at any suitable temperature below the boiling point of the liquid

constituents, below 212° F. in the case of aqueous baths, preferably at about room temperature.

A typical dyeing bath for glass fiber fabrics contains as solids from 0.02 to 5% pigment, from 0.005 to 5% cationic flocculating agent, from 0.25 to 5% of resin binder, from 0.03 to 3% non-slip agent, and from 0.5 to 5% abrasion resistant additive. The rest of the bath is water, i.e., the water content of the bath is from 77% to 99.195%.

10 A typical dyeing bath for other fabrics, including the synthetic fabrics, contains from 0.25 to 5% resinous binder, from 0.02 to 5% pigment, and from 0.005 to 5% cationic flocculating agent; the rest of the bath is water, but may be methanol, ethanol, isopropyl alcohol, or acetone. Thus the liquid content of the bath is from 85% to 99.725% by weight.

In producing the dyeing baths for the practice of the process of this invention, only a portion of the dispersed anionically charged pigments and finish constituents, if present, need be flocculated by the flocculating agent, leaving up to 50-90% of the pigment in the bath in finely dispersed non-agglomerated form. In such case, the flocculated or agglomerated pigment particles color chiefly or only the loosely constructed or float areas of the fabric, whereas the finely dispersed particles color the more tightly constructed or background areas of the fabric. By variation of the amount of the pigment agglomerated, and hence the concentration of the agglomerated pigment particles in the bath, different tonal effects are obtained. Similarly, by varying the concentration of the non-agglomerated pigment particles in the bath, different tonal background effects are obtained.

Alternatively, substantially all of the anionic pigment in a bath can be agglomerated or flocculated by the flocculating agent. The resultant bath functions to tone the loosely constructed fabric areas substantially to the exclusion of the more tightly woven portions thereof, leaving a substantially white background in the tightly woven areas to provide a sharply contrasting toned pattern when white fabrics are dyed; the original colored background is left undyed when colored fabrics are dyed by the process of this invention using such bath.

Still another procedure, according to the invention, involves adding to about 20-40%, preferably about 30%, of the total volume of dye bath, pigment particles for coloration of the relatively loosely constructed areas of the fabric, adding to this portion of the bath a cationic flocculating agent, then adding the remainder of the volume of the bath to the resulting mixture and introducing into the bath thus produced an additional finely dispersed pigment, if desired, of a different color from that employed initially. This finely dispersed pigment remains suspended in the bath in a non-agglomerated form. When the fabric is padded through this bath, multi-color effects are obtained, the agglomerated pigment particles dyeing essentially the relatively loosely constructed areas of the fabric and the dispersed non-agglomerated pigment particles dyeing the background or tightly constructed areas thereof.

60 The fabric on leaving the bath is passed through the padding or squeeze rollers, which squeezes out the dyeing liquor and causes it to flow over the fabric. During such flow the loosely constructed areas tend to trap the agglomerated pigment particles usually containing resin binder particles and other particles such as colloidal silica and abrasion resistant agent, if present, and cause the agglomerates to remain thereon while leaving the tightly constructed areas substantially free of the agglomerates. As 65 the fabric passes through the padding rollers, the agglomerates are pressed into the loosely constructed areas and upon subsequent curing are bonded thereto. Employing a bath also containing non-agglomerated pigment particles, such particles adhere for the most part 70 preferentially to the tightly constructed areas; while the 75

agglomerates are washed by the back-flow of liquid from such tightly constructed areas, the non-agglomerated colloidal pigment particles remain thereon. It will be understood that the above is offered as an explanation of why the present invention results in selective dyeing or two-tone dyeing and the invention is not to be limited to this explanation.

When treating long yardage, the agglomerated pigment in the bath is replenished from time to time, or continuously. Also a suspension of the non-agglomerated pigment particles may be added to the bath from time to time, or continuously, when coloring of the background area is desired to produce the desired shade or shades.

In the case of glass fiber fabrics, the average wet pickup after leaving the squeeze rollers is 20 to 90% based on the weight of the fabric, depending upon the amount of textured, bouclé, filament, or other yarns of relatively loose construction in the fabric. In the case of cellulosic fabrics, particularly rayons, the average wet pickup after leaving the squeeze rollers is within the range of 60-75% based upon the weight of the fabric.

The fabric after leaving the squeeze rollers of the padder is passed through a drying or curing oven where it is subjected to temperatures of from 250 to 375° F. for from one to ten minutes. The longer times are used when heating at the lower temperatures or with high wet pickup fabrics and the shorter residence times when heating at the higher temperatures within this range.

If desired, when dyeing glass fiber fabrics, the fabrics are given a water-repellent treatment with a stearato-chromyl chloride or other Werner complex in which the acids group coordinated with the chromium atom has more than 10 carbon atoms, as described in United States Patents 2,273,040 and 2,356,161. The water-repellent is applied by passing the fabric through a bath containing from 0.2 to about 4 or 5% by weight chrome complex and then drying at 250-375° F. to set the water-repellent material on the fabric.

The following examples are given to illustrate specific embodiments of the dyeing process and bath of the invention. It will be appreciated that the invention is not limited to these examples.

#### Example I

A dyeing bath in amount of 48 gallons was prepared containing 3% colloidal silica (Syton DS added to the bath as a suspension of 30% of colloidal silica in water); 2% polytetrafluoroethylene (Teflon); 2½% polyethyl acrylate (Hycar 4501), the rest being water. The ingredients were mixed at 70° F. and the bath was then divided into two portions, one containing 30% of the bath by volume, and the other 70%. To the 30% portion was added 1 lb. of iron oxide yellow (Interchemical Corporation's Padding Yellow K-9850), and 0.84 lb. of phthalocyanine pigment (Interchemical Corporation's Padding Green B-9450) in the form of aqueous anionic pigment dispersions. The resultant mixture was stirred vigorously to disperse the pigment.

Six pounds of a 1% Kylan solution (containing the acetic acid salt of deacetylated chitin) were prepared by dissolving 0.06 lb. of Kylan flakes in 5.94 lbs. of 1% acetic acid. 5.6 lbs. of the Kylan solution was added slowly to the 30% bath portion; upon addition the pigment and finish (Teflon and Syton) particles agglomerated. The 30% bath portion thus produced was remixed with the 70% portion.

A glass fiber fabric comprising float areas of bulked yarn and background areas of filament yarn was passed through this bath at the rate of 39 feet per minute. The pickup was 32%. Thereafter the fabric was passed through a drying oven at 330° F. for a residence time of 2.3 minutes.

The fabric was dyed a brilliant mint green in the float portions; the background portions remained unstained white.

#### Example II

This example differs from Example I chiefly in that after the pigments and flocculating agent were added to the 30% volume, and the 30% and 70% volumes of the bath were combined, 0.99 lb. of indanthrene vat dye (Interchemical's Padded Yellow N-9851), and 2.82 lbs. of a second indanthrene vat dye (Interchemical's Padding Brown 9500-21) thoroughly mixed in a gallon of water were added to the dyeing bath.

A glass fiber fabric similar to that processed in Example I was dyed and finished in the same manner as the fabric in Example I. The float portions of the fabric were dyed a brilliant mint green and the background portions a champagne shade.

#### Example III

The bath in this example was made by adding 4 lbs. of metal oxide pigment (Drakenfeld's turquoise 10107) to 10 gallons of water. 2.4 lbs. of Nalco D-1535 was heated

until the opaqueness disappeared and then slowly added to the pigment dispersion while stirring. The heating of the Nalco was for the purpose of dissolving lumps, the cold material could be added with the same results provided the mixture was stirred enough to eliminate lumps. Enough water was added to make a volume of 48 gallons thus obtaining a bath containing approximately 1% of agglomerated pigment. 1.6 lbs. of polyvinyl acetate emulsion was added to the bath.

An all-glass fiber fabric containing filament and bulked yarns was padded through this bath at a speed of 30 feet per minute; fabric wet pickup was 90%. The fabric was then dried at 320° F. with a residence time in the dryer of three minutes. It was then padded through a second bath containing 4% Syton and 3% Rhoplex HA-4 binder to impart to the fabric a deluster and crock and wash-fast finish. The fabric was then dried at 300° F. with a dwell time of three minutes in the dryer. The bulked yarns in the fabric were colored a bright turquoise and the filament yarns remained white.

#### Example IV

Into the 20% portion of a 48 gallon bath containing Hycar, Syton and Teflon, as in Example I, was dispersed 8 lbs. of phthalocyanine (Interchemical's Padding Green B-9450) and 0.12 lb. of carbon black (Interchemical's Padding Grey 2K-9250). To this dispersion was slowly added with agitation 1 lb. of Lyofix EW and 2 lbs. of a 1% Kylan solution. The resultant 20% bath portion was then combined with the remaining 80% by volume.

An all-filament glass fabric having raised float yarn was padded through this bath at a speed of 39 feet per minute with a wet pickup of 25%. The fabric was dried at 330° F. with a residence time of 2.3 minutes in the dryer. Fabric having a brilliant green tipped effect on the raised float yarns and a faint neutral green tint on the background portions resulted.

#### Example V

The bath in this example contained 1% yellow iron oxide in 10% water, 1% Kylan solution, 0.5% melamine formaldehyde resin, and about 87.5% methanol. The bath was produced by placing the dispersion of the dye in water in a container, adding the methanol and the Kylan, mixing until agglomerates resulted, and then adding the melamine resin to the resultant bath.

Upon padding an all-glass fiber fabric having bulked yarn through this dye bath and curing the fabric as in Example I, a two-tone fabric resulted having the bulked yarns colored a bright yellow and the background areas an off-white shade.

Upon repetition of this example, substituting a dye dispersion in methanol for the water in which the dye had been dispersed, and thus employing a bath substantially free of water, the contrast in color was appreciably more marked. The use of ethanol, and iso-

propyl alcohol instead of the methanol gives comparable results.

*Example VI*

This example involved the use of dry powder pigments instead of dispersions, as in the preceding examples.

Cobalt blue was pasted in water and the resultant paste dispersed in 20% of the total volume of the bath.

4 ml. of a 1% solution of Kylan was then added. The remaining 80% by volume of the bath was then mixed with the 20%, the former containing 2% Hycar-4501. Upon producing the bath in this manner, satisfactory agglomerates of the pigment resulted as evidenced by the dyeing of a glass fiber fabric having bulked yarns in this bath by passage therethrough and after treatment, as in Example I; the dyed fabric had a light blue shade in the bulked yarn areas while the background areas remained white having only a slight tint.

*Example VII*

Into 20% of a 48 gallon bath was added 0.8 lb. of Hycar, 1.6 lbs. of Syton, and 4 lbs. of indanthrene vat dye (Interchemical's Padding Yellow N-9851) and the mixture stirred to disperse the dye particles. To this dispersion was added 9.82 lbs. of a 1% Kylan solution prepared as in Example I. The remaining 80% of the water content of the bath was then added and 8 lbs. of Moropol ARF resin binder introduced into the bath.

A synthetic fabric consisting of 100% spun rayon having floats was padded through this bath at a speed of 15 yards per minute, with a wet pickup after leaving the padding rolls of 73% by weight. The fabric was dried at 330° F. with a residence time of two minutes in the dryer. The float areas of the fabric were colored a golden yellow and the background portions a much lighter shade of yellow.

It will be noted that the present invention provides a process and dyeing bath for selectively dyeing fabrics having different surface structures or characteristics, simply and economically, and for producing desired tonal effects. The invention is particularly useful in dyeing bulked, bouclé, or filament glass fiber fabrics producing contrasting shades or tones on the bulked or loosely constructed areas as compared with those in the tightly constructed, usually the background areas.

Heretofore to produce multi-colored glass fiber fabrics, it was necessary to use pre-dyed fibers dyed with colorants able to withstand temperatures of 1200° to 1300° F. The present invention can be practiced with pigments or anionic pigment dispersions having melting or decomposition points above the temperature of the drying or curing, which temperature depends upon the residence time in the curing or drying zone and may be as low as 200° F. and in general is from 300 to 400° F. Thus the present invention permits of a much greater choice of pigments to produce a vastly larger range of shades and colors.

All percentages employed in this specification, unless otherwise specified, are given on a weight basis.

Since different embodiments of the invention may be made without departing from the scope thereof, it is intended that all matter contained in the above description shall be interpreted as illustrative and not in a limiting sense.

What is claimed is:

1. A process for coloring glass fiber fabrics having relatively tightly and loosely constructed surfaces, which comprises forming a padding bath containing at least 77% by weight of liquid, from 0.005% to 5% by weight of a cationic flocculating agent from the group consisting of deacetylated chitin; polyalkyl-polyamines; polyalkyl-polyamine fatty acid reaction products; amino aldehyde condensate dye-fixatives; methylchloride quaternary of the stearic acid amide of 1-(2-aminoethyl) 2-heptadecenyl-2-imidazoline; fluid oil in water type emulsions of low molecular weight polyethylene chemically stabilized with a cationic amine acetate derivative of a long chain fatty compound; dicyandiamine formaldehyde dye fixatives; colloidal cationic thermo-setting resinous reaction products of straight chain poly-functional amines and an aldehyde; and a mixture of such agents, from 0.02% to 5% by weight of anionic pigment particles and binder for said pigment particles, the amount of said cationic flocculating agent within said range being sufficient to effect the flocculation of at least a substantial proportion of said pigment particles, maintaining the solid constituents of said bath including the flocculated pigment particles suspended and uniformly dispersed throughout said bath, padding the glass fiber fabric through said bath to deposit the flocculated pigment particles preferentially on the loosely constructed surfaces leaving the tightly constructed surfaces substantially free of said flocculated pigment particles, and thereafter heating the fabric to cause the binder to bond the flocculated pigment particles to the loosely constructed surfaces to produce contrasting tonal effects on the respective tightly constructed and loosely constructed surfaces of said glass fiber fabric.

2. The process as defined in claim 1, in which the anionically charged pigment particles initially have a particle size of from 0.007 to 40 microns and upon flocculation produce agglomerates having an average particle size of from 10 to 2000 microns.
3. A process for coloring glass fiber fabrics having relatively tightly and loosely constructed surfaces, which comprises forming a padding bath containing at least 77% by weight of water, from 0.005% to 5% by weight of a cationic flocculating agent from the group consisting of deacetylated chitin; polyalkyl-polyamines; polyalkyl-polyamine fatty acid reaction products; amino aldehyde condensate dye-fixatives; methylchloride quaternary of the stearic acid amide of 1-(2-aminoethyl) 2-heptadecenyl-2-imidazoline; fluid oil in water type emulsions of low molecular weight polyethylene chemically stabilized with a cationic amine acetate derivative of a long chain fatty compound; dicyandiamine formaldehyde dye fixatives; colloidal cationic thermo-setting resinous reaction products of straight chain poly-functional amines and an aldehyde; and a mixture of such agents, from 0.02% to 5% by weight of anionic pigment particles, and from 0.25% to 5% by weight of resin binder, agitating said bath to effect the flocculation of at least a substantial portion of said pigment particles in said bath by the cationic flocculating agent and to maintain the flocculated pigment particles and resin binder suspended in and uniformly distributed throughout said bath, padding the glass fiber fabric through said bath thereby preferentially depositing on the loosely constructed surfaces flocculated pigment particles and resin binder with substantially no deposition of said flocculated pigment particles on the tightly constructed surfaces, and thereafter heating the fabric to effect the bonding of the flocculated pigment particles to the loosely constructed surfaces by the resin binder and thus producing contrasting tonal effects on the loosely and tightly constructed surfaces.
4. The process as defined in claim 3, in which the amounts of cationic flocculating agent and anionic pigment are proportioned so that substantially all of the pigment is flocculated by the cationic flocculating agent and only the loosely constructed surfaces are colored with said pigment.
5. The process as defined in claim 3, in which after the formation of said bath by mixing said cationic flocculating agent, aqueous dispersion of pigment particles, resin binder and water, a dispersion of a pigment of a different color than the first mentioned pigment having a particle size smaller than that of the flocculated pigment particles is added to the bath and upon padding the fabric through said bath the flocculated pigment par-

## 11

ticles are deposited on the loosely constructed surfaces and the said pigment of different color is deposited on the tightly constructed surfaces.

6. A process for coloring glass fiber fabrics woven to provide tightly and loosely constructed surfaces, which process comprises, producing a padding bath containing from 0.05% to 5% by weight of a cationic flocculating agent from the group consisting of deacetylated chitin; polyalkyl-polyamines; polyalkyl-polyamine fatty acid reaction products; amino aldehyde condensate dye-fixatives; methylchloride quaternary of the stearic acid amide of 1-(2-aminoethyl) 2-heptadecenyl-2-imidazoline; fluid oil in water type emulsions of low molecular weight polyethylene chemically stabilized with a cationic amine acetate derivative of a long chain fatty compound; dicyandiamide formaldehyde dye fixatives; colloidal cationic thermo-setting resinous reaction products of straight chain poly-functional amines and an aldehyde; and a mixture of such agents, from 0.02% to 5% by weight of anionic pigment particles, from 0.25% to 5% of a binder resin and at least 85% by weight of water, in which bath at least a substantial proportion of the anionic pigment is in an agglomerated condition, agitating said bath to maintain the agglomerated pigment particles in suspension and dispersed uniformly throughout said bath, padding said glass fiber fabric through said bath to deposit preferentially on the loosely constructed surfaces the agglomerates of said pigment particles and resin binder, and thereafter heating the fabric to a temperature to cause the resin binder to bond the agglomerated pigment particles to the loosely constructed surfaces, thus coloring the loosely constructed surfaces preferentially to the tightly constructed surfaces.

7. The process as defined in claim 6, in which an aqueous dispersion of a second pigment having a different color from that of the first mentioned pigment is added to the bath and dispersed therein, upon padding the glass fiber fabric through the resultant bath the loosely constructed surfaces have deposited thereon the said agglomerates of the pigment particles admixed with resin binder and the tightly constructed surfaces have deposited thereon the second mentioned pigment admixed with resin binder, and upon heating the thus treated fabric the pigment agglomerates are bonded to the loosely constructed surfaces and the second mentioned pigment to the tightly constructed surfaces.

8. The process as defined in claim 6, in which the bath also contains from .3% to 4% by weight of colloidal silica, from 5% to 5% by weight of polytetrafluoroethylene and the fabric after padding through said bath is heated to a temperature of from 200° to 400° F. for from 1 to 10 minutes.

9. A process for coloring glass fiber fabrics woven to provide tightly and loosely constructed surfaces, which process comprises, mixing with at least 77% by weight of water a dispersion of anionically charged pigment particles having a particle size of from 0.007 to 40 microns, a cationic flocculating agent from the group consisting of deacetylated chitin; polyalkyl-polyamines; polyalkyl-polyamine fatty acid reaction products; amino aldehyde condensate dye-fixatives; methylchloride quaternary of the stearic acid amide of 1-(2-aminoethyl) 2-heptadecenyl-2-imidazoline; fluid oil in water type emulsions of low molecular weight polyethylene chemically stabilized with a cationic amine acetate derivative of a long chain fatty compound; dicyandiamide formaldehyde dye fixatives; colloidal cationic thermo-setting resinous reaction products of straight chain poly-functional amines and an aldehyde; and a mixture of such agents, and a resin binder to produce a padding bath containing from .02% to 5% by weight of said pigment particles in which at least a substantial proportion of said pigment particles is agglomerated and the agglomerates have an average particle size

## 12

of from 10 to 2000 microns, from .005% to 5% by weight of said cationic flocculating agent, from 0.25% to 5% by weight of said resin binder, and at least 77% by weight of water, agitating said padding bath to maintain said agglomerated pigment particles in suspension therein and uniformly dispersed therethrough, padding the fabric through said bath thereby preferentially depositing on the loosely constructed surfaces flocculated pigment particles and resin binder with substantially no deposition of said flocculated pigment particles on the tightly constructed surfaces, and thereafter heating the fabric to effect the bonding of the flocculated pigment particles to the loosely constructed surfaces by the resin binder and thus producing contrasting tonal effects on the loosely and tightly constructed surfaces.

10. A process for coloring glass fiber fabrics woven to provide tightly and loosely constructed surfaces, which comprises, forming a padding bath by mixing with about 20% to 40% of the volume of said bath a dispersion of anionic pigment particles, a cationic flocculating agent from the group consisting of deacetylated chitin; polyalkyl-polyamines; polyalkyl-polyamine fatty acid reaction products; amino aldehyde condensate dye-fixatives; methylchloride quaternary of the stearic acid amide of 1-(2-aminoethyl) 2-heptadecenyl-2-imidazoline; fluid oil in water type emulsions of low molecular weight polyethylene chemically stabilized with a cationic amine acetate derivative of a long chain fatty compound; dicyandiamide formaldehyde dye fixatives; colloidal cationic thermo-setting resinous reaction products of straight chain poly-functional amines and an aldehyde; and a mixture of such agents, to produce a dispersion of agglomerates of said pigment particles in water, adding the dispersion of agglomerated pigment particles to the remaining 60% to 80% of the volume of said bath, incorporating in said bath a resin binder, then adding to said bath a dispersion of anionic pigment particles of a different color, the said pigments, cationic flocculating agent, water and binder being introduced into said bath in amounts to produce in the total bath, by weight, from .005% to 5% of said cationic flocculating agent, from .02 to 5% by weight of said pigments, from 0.25% to 5% by weight of said resin binder and at least 77% by weight of water, agitating said bath to maintain said flocculated pigment particles and the said pigment particles of different color suspended therein and uniformly dispersed throughout said bath, padding said glass fiber fabric through said bath to deposit the said pigment agglomerates and resin binder upon the loosely constructed surfaces and the said pigment particles of different color and resin binder upon the tightly constructed surfaces, and thereafter heating the fabric to cause the resin binder to bond the agglomerated pigment particles to the loosely constructed surfaces and the pigment particles of different color to the tightly constructed surfaces.

11. The process as defined in claim 10, in which the said padding bath contains from .05% to 1% by weight of said cationic flocculating agent, from .05% to 4% by weight of said pigment, from .05% to 2% by weight of resin binder, from 0.6% to 2% of colloidal silica, and from 0.5% to 5% polytetrafluoroethylene, the agglomerated particles have a particle size of from 10 to 2000 microns, and the pigment particles of a different color have a particle size of from 0.007 to 40 microns.

65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
79

UNITED STATES PATENT OFFICE  
CERTIFICATE OF CORRECTION

Patent No. 3,108,897

October 29, 1963

William L. Hamiter et al.

It is hereby certified that error appears in the above numbered patent requiring correction and that the said Letters Patent should read as corrected below.

Column 5, line 27, for "ethyl methacrylate" read -- ethyl ethacrylate --; line 43, for "pigments" read -- pigment --.

Signed and sealed this 14th day of April 1964.

(SEAL)

Attest:

ERNEST W. SWIDER

EDWARD J. BRENNER

Attesting Officer

Commissioner of Patents